

## UNITED STATES PATENT OFFICE

2,596,485

## TITANIUM BASE ALLOY

Robert I. Jaffee and Horace R. Ogden, Columbus, Ohio, assignors, by mesne assignments, to Remington Arms Company, Inc., Bridgeport, Conn., a corporation of Delaware

No Drawing. Application December 2, 1950,  
Serial No. 198,917

4 Claims. (Cl. 75—134)

1

This invention relates to titanium base alloys, and contemplates certain structurally useful quaternary alloys of titanium with aluminum, chromium and molybdenum, as well as a process for the preparation of such alloys in a ductile condition.

In application of Jaffee and Ogden, Serial No. 122,577, filed October 20, 1949, now Patent No. 2,554,031, issued May 22, 1951, there are disclosed certain structural alloys containing aluminum and molybdenum. In the application of Jaffee and Ogden, Serial No. 122,576, filed October 20, 1949, there are disclosed certain ductile alloys of titanium with aluminum and chromium; also several alloys of titanium and aluminum with relatively small amounts of chromium and molybdenum. The present application is a continuation-in-part of Application Serial No. 122,576.

The titanium base metal used in the present alloys may contain substances or impurities besides titanium, as normally found in either high purity titanium or commercially pure titanium. It may be, for example, a high purity or "iodide" process titanium, as produced according to the Van Arkel U. S. Patent No. 1,671,213. Alternatively, it may be a commercial titanium, as produced, for example, by magnesium-reduction processes, such as the process of U. S. Patent No.

0.5%, if the alloys are to possess good ductility as cast or as worked and annealed.

It has been found, however, that the presence of a small amount of carbon, say 0.05% to 0.3%, with or without 0.01% to 0.15% nitrogen or 0.01% to 0.25% oxygen, or both oxygen and nitrogen, may be beneficial. Among the alloys of this invention are those made either with a commercial titanium base meeting such specifications, or with a high purity titanium base containing similar amounts of added carbon, oxygen and/or nitrogen. Thus, within the purview of the invention are quaternary alloys containing from about 2% to about 5% aluminum, 1% to 6% chromium and 1% to 6% molybdenum, as additions to a titanium base which may be of high purity or may contain up to 0.15% nitrogen, 0.25% oxygen and/or 0.3% carbon; the total nitrogen, oxygen and carbon content preferably not exceeding 0.5%. These alloys are of high tensile strength, and of such ductility as to permit their forming and fabrication by the usual metallurgical processes, such as rolling, drawing and forging. If the combined content of chromium and molybdenum is relatively low, say about 2.5%, the alloy may be prepared for use by quenching from a temperature of 850° C. to 950° C., and thereafter annealing. Typical alloys of this group, and their properties, are as follows:

## Tensile properties

| Composition<br>(Balance—Ti)                                                                                                                                                                             | Annealed<br>Hardness     | Propor.<br>Limit                        | 0.1%<br>Offset                          | 0.2%<br>Offset                          | Ulti-<br>mate<br>Strength                | Per<br>Cent<br>Elonga-<br>tion in 1" | Per<br>Cent<br>Area<br>Reduc-<br>tion |
|---------------------------------------------------------------------------------------------------------------------------------------------------------------------------------------------------------|--------------------------|-----------------------------------------|-----------------------------------------|-----------------------------------------|------------------------------------------|--------------------------------------|---------------------------------------|
| Al, 5.0<br>Mo, 1.25<br>Cr, 1.25<br>Al, 5.0<br>Mo, 1.25<br>Cr, 1.25<br>C, 0.25<br>Al, 5.0<br>Mo, 1.25<br>Cr, 1.25<br>C, 0.25<br>O, 0.1<br>Al, 5.0<br>Mo, 1.25<br>Cr, 1.25<br>C, 0.25<br>O, 0.1<br>N, 0.1 | 288<br>347<br>364<br>391 | 83,000<br>131,000<br>134,000<br>155,000 | 91,000<br>142,000<br>143,000<br>161,000 | 91,000<br>142,000<br>144,000<br>161,000 | 107,000<br>147,000<br>156,000<br>161,000 | 12<br>—<br>9<br>—                    | 27<br>26<br>11<br>20                  |

2,205,854, to Kroll, or modifications thereof; provided that the carbon, oxygen and nitrogen contents of these alloys, hence of the base metal, should not exceed 0.5%, 0.25% and 0.15% respectively, nor should they total more than about

Quaternary alloys having a higher content of molybdenum and/or chromium, as quenched from the all-beta field, possess acceptable ductility, but are severely embrittled by subsequent exposure to moderately elevated temperatures.

Hitherto it has been believed that alloys containing for example 5% aluminum and 4% each of chromium and molybdenum were inherently too brittle for structural use. It has been found, however, that if such alloys are slowly cooled from a temperature high in the two-phase field or within the all-beta field, say 850° C. to 950° C., they are not only ductile as cooled but substantially retain their ductility after prolonged exposure to temperatures as high as 400° C. In a typical processing, the alloy is heated to 900° C., and retained at this temperature for about three-quarters of an hour. Thereafter, it is cooled at a rate of about 1° per minute to a temperature of about 500° C., after which cooling may be more rapid. The soaking may be performed in an electric furnace and, after soaking, the furnace control set back 60° every hour until the temperature is below about 500° C., after which the heat is turned completely off, the work remaining in the furnace until both are reduced substantially to room temperature. The resulting alloys are not only ductile but remain ductile upon subsequent exposure to elevated temperatures such as 300° or 400° C. The slow cooling has the effect of transforming a maximum amount of the metal from the high temperature beta-phase to the low temperature alpha-phase, thus avoiding the embrittling coherency hardening brought about by the aging transformation of the unstable beta of quenched alloys.

"Bend ductility" is a more severe and practical test of utility than is tensile elongation. Bend ductility is measured as the radius, expressed as a multiple of specimen thickness, at which the specimen can be bent to an angle of 75° without fracture.

Typical alloys within the present invention, their hardness and bend ductility, as cooled in the manner above described and after elevated temperature exposure, are as follows:

*Delayed cooling from 900° C.*

| Composition (Balance—Ti) | Before Storage:  |             | Stored 64 Hrs. at 300° C.: |             | Stored 200 Hrs. at 400° C.: |             |
|--------------------------|------------------|-------------|----------------------------|-------------|-----------------------------|-------------|
|                          | Vickers Hardness | Bend Radius | Vickers Hardness           | Bend Radius | Vickers Hardness            | Bend Radius |
|                          |                  | T           |                            | T           |                             | T           |
| Al, 5.0                  |                  |             |                            |             |                             |             |
| Mo, 2.5                  | 355              | 2.0         | 362                        | 2.2         | 382                         | 6.7         |
| Cr, 2.5                  |                  |             |                            |             |                             |             |
| Al, 5.0                  |                  |             |                            |             |                             |             |
| Mo, 2.5                  | 345              | 2.2         | 377                        | 2.0         | 375                         | 2.9         |
| Cr, 2.5                  |                  |             |                            |             |                             |             |
| C, 0.05                  |                  |             |                            |             |                             |             |
| Al, 5.0                  |                  |             |                            |             |                             |             |
| Mo, 4.0                  | 336              | 1.1         | 374                        | 2.0         | 398                         | 2.5         |
| Cr, 4.0                  |                  |             |                            |             |                             |             |
| Al, 5.0                  |                  |             |                            |             |                             |             |
| Mo, 4.0                  | 347              | 2.2         | 390                        | 2.0         | 385                         | 8.1         |
| Cr, 4.0                  |                  |             |                            |             |                             |             |
| C, 0.05                  |                  |             |                            |             |                             |             |
| Al, 5.0                  |                  |             |                            |             |                             |             |
| Mo, 6.0                  | 352              | 3.1         | 410                        | 5.9         | 428                         | 7.6         |
| Cr, 6.0                  |                  |             |                            |             |                             |             |
| C, 0.05                  |                  |             |                            |             |                             |             |

It will be seen that not only are these alloys ductile in the slow cooled condition, but that they largely retain their ductility after as much as 200 hours storage at 400° C. The same alloys in as quenched condition show hardness and ductility comparable with the slow cooled condition, but storage for 64 hours at 300° C., raises average Vickers hardness well over 100 points and virtually destroys all bend ductility. It is thus in slow-cooled, or slow-cooled and aged condition, that the alloys find their greatest utility.

What is claimed is:

1. A ductile alloy consisting essentially of 2% to 5% aluminum, 1% to 6% chromium, 1% to 6% molybdenum, balance titanium.
2. A ductile alloy consisting essentially of 2% to 5% aluminum, 1.25% chromium, 1.25% molybdenum, balance titanium.
3. A ductile alloy consisting essentially of 2% to 5% aluminum, 2.5% chromium, 2.5% molybdenum, balance titanium.
4. A ductile alloy consisting essentially of 2% to 5% aluminum, 4% chromium, 4% molybdenum, balance titanium.

ROBERT I. JAFFEE.  
HORACE R. OGDEN.

**REFERENCES CITED**

The following references are of record in the file of this patent:

**UNITED STATES PATENTS**

| Number    | Name          | Date          |
|-----------|---------------|---------------|
| 2,188,765 | Young         | Jan. 30, 1940 |
| 2,487,367 | Austin        | Apr. 19, 1949 |
| 2,490,571 | Anicetti      | Dec. 6, 1949  |
| 2,554,031 | Jaffee et al. | May 22, 1951  |